

# UNITED STATES PATENT OFFICE.

LÉONIE VON JARACZEWSKI, GEB. STERN, OF BERLIN, GERMANY.

## PROCESS FOR THE PRODUCTION OF A FILTER-STUFF BY THE EMPLOYMENT OF COAL OR SIMILAR FILTER MATERIALS.

1,147,991.

Specification of Letters Patent. Patented July 27, 1915.

No Drawing.

Application filed October 6, 1913. Serial No. 793,755.

*To all whom it may concern:*

Be it known that I, LÉONIE VON JARACZEWSKI, née STERN, a subject of the Emperor of Germany, residing at 8 Lennéstrasse, Berlin, W., Germany, formerly Oels, have invented certain new and useful Improvements in Processes for the Production of a Filter-Stuff by the Employment of Coal or Similar Filter Materials, of which 10 the following is a specification.

This invention has for its object a process for producing filter material from bone-black.

Hitherto filters from bone-black have 15 been made by compressing the bone-black into slabs by air pressure. As however the fine particles of the bone-black do not bind together directly, a special binding medium was required for the manufacture of such 20 filter slabs whereby the bone-black loses some of its considerable filtering properties.

The new process consists essentially in precipitating bone-black in the hot water bath on a tissue which is easily permeable 25 and has a hairy surface. The fibers of the tissue are loosened to a certain extent in the hot water bath so that the gaps between the fibers and the pores of the tissue get larger, the precipitate of bone-black being able to 30 penetrate deeply into the tissue. After partial cooling, a second deposit of fibrous material is precipitated on the tissue and the filter thus formed is finally dried by heating and compressed, whereby a felting of the 35 upper layer of fibers with the lower layer of tissue is effected, the intermediate layer of bone-black being securely embedded between the two layers of fibers interlaced and clinging together. The upper and lower 40 layers of fibers have a purely mechanical effect, while the intermediate layer of bone-black exerts the well known chemical or physical action upon the liquid to be filtered.

An example of the application of the new 45 process is the following:—A tissue having a fine hairy surface (fustian or the like) is placed in a boiling pot, the hairy side turned up, for each square meter of tissue 50 200 grams of water are mixed with 50 grams of alcohol, and 30 grams of bone-black; this mixture is poured on the tissue, and boiled for 5 minutes in the closed boiling pot whereupon it is left to cool. The tissue

is then taken out and left to dry for several 55 hours without being wrung out so that it gets half dry. It is then placed between two sheets of hard glazed paper and treated with a hard roller heated by hot water or steam until it is perfectly dry. The tissue is then 60 placed upon a sieve, the hairy surface and the deposit of bone-black being turned up.

50 grams of bone-black, 15 grams of asbestos in fine flakes, 10 grams of cellulose are dissolved in one liter of water and the 65 solution is uniformly poured on the tissue which has just been spread out. If the water which flows off the tissue shows a yellowish color, cold water must be poured repeatedly on the tissue to wash out the coloring 70 matter. It will be seen at this stage already that the preliminarily boiled tissue does not let the bone-black pass through it. If the water flows off quite clear the sieve with the tissue is stored in a heated room 75 to dry rapidly and is then brought under a press before it has been completely dried, either again between two sheets of glazed paper or between two polished metal plates, and it is then left in the press for several 80 hours. The tissue, after having been taken out of the press, is again rolled with a heavy cold roller.

By this process there is not only obtained 85 an absolutely secure binding of a layer of bone-black which is sufficiently finely distributed in the tissue, but also an intimate fine interlacing of the asbestos with the hair of the filter material, whereby a filtering 90 felt is produced of form and intimate fineness hitherto not obtainable.

I claim:—

A process for producing a filtering material consisting in boiling for five minutes 95 a tissue with fine hairy surface in a solution of 50 grams of alcohol and 30 grams of bone-black, in drying said tissue, in placing the tissue on a sieve the hairy surface turned up, in uniformly pouring on the tissue a solution of 50 grams of bone-black, 15 grams of asbestos in fine flakes and 10 grams of cellulose and in drying said tissue under pressure, substantially as described and shown and for the purpose set forth.

In testimony whereof I have affixed my 100 105 signature, in presence of two witnesses.

LÉONIE VON JARACZEWSKI, GEB. STERN.